

# UNITED STATES PATENT OFFICE.

ROBERT H. HENDERSON, OF EAST ORANGE, NEW JERSEY, ASSIGNOR TO WESTINGHOUSE LAMP COMPANY, A CORPORATION OF PENNSYLVANIA.

## PROCESS OF TREATING INCANDESCENT-LAMP FILAMENTS.

1,086,171.

Specification of Letters Patent.

Patented Feb. 3, 1914.

No Drawing.

Application filed December 5, 1910. Serial No. 595,631.

*To all whom it may concern:*

Be it known that I, ROBERT H. HENDERSON, a citizen of the United States, and a resident of East Orange, in the county of 5 Essex and State of New Jersey, have invented a new and useful Improvement in Processes of Treating Incandescent-Lamp Filaments, of which the following is a specification.

10 My invention relates to certain improvements in the manufacture of incandescent electric lamps, the object being to produce incandescent lamps having filaments of higher efficiency and greater durability than obtained by the usual processes.

15 The invention is particularly applicable to filaments composed of or containing tungsten.

In the manufacture of incandescent lamps 20 consisting of tungsten or similar materials, the ordinary process consists in squirting the filament from a paste and sintering the metallic particles together by heating the filament to a temperature about the equivalent 25 of the temperature at which the filament is to be run in the finished lamp. The filament thus prepared is then introduced into the lamp bulb and the latter is exhausted of air, the filament being heated during this 30 operation to approximately the same or a little higher than the temperature it will have while burning in the finished lamp. This procedure is followed when the lamps are exhausted with mercury pumps which 35 give a very high vacuum. When the exhaust process is conducted by means of oil vacuum pumps which give a lower vacuum, it has been customary to follow the same procedure as in the manufacture of carbon 40 lamps, namely to introduce a small amount of phosphorus vapor into the bulb just before the lamp is sealed off from the pump for the purpose of obtaining a higher vacuum. No attempt is made, however, to produce 45 any reaction between the phosphorus vapor and the filament.

The completed filament is at best but imperfectly sintered together and represents merely a mass of metallic particles superficially welded and sintered together and 50 after the lamp is exhausted it is necessary to subject it to an aging process which consists in burning it for a certain period at its normal voltage and during this operation

the filament undergoes a further sintering. 55 Examined under the microscope such filament does not present a smooth surface but has a rather rough and pitted appearance.

It is well understood in the manufacture 60 of lamps that a filament with a smooth surface is superior to one with a rough surface as far as its luminous efficiency and light emissivity is concerned. It is desirable, therefore, that means be found for producing the tungsten or like filament with a 65 much more smooth exterior than obtained by processes heretofore proposed. I find that when the filament is heated to a very high temperature in a high vacuum, its surface is somewhat improved, but if at that 70 high temperature it is surrounded with an atmosphere of gas or vapor such for instance as phosphorus, a marked improvement is obtained and a filament is produced which, under the microscope, appears much more 75 smooth and brilliant. This smoothness of surface may be due to a fluxing of the metallic particles at the surface of the filament as their appearance is as though they were caused to flow together under the combined 80 action of the high temperature and the gas or vapor. This may possibly be due to the intermediate formation of an alloy or compound of the metallic particles and the gas, at the surface of the filament, which alloy 85 or compound is immediately decomposed. I do not, however, desire to be understood as giving this explanation as necessarily 90 the correct one, but it is advanced as being a probable explanation.

The filament may be dipped into a suitably prepared emulsion of the reacting element or a suitable compound thereof, or the reacting gas may be obtained by directly vaporizing a sufficient quantity of the element or of a suitable compound thereof. 95

I prefer to carry out this process in conjunction with the ordinary process of exhausting the lamp of air. Thus, for instance, after the lamp has undergone the 100 regular process of exhaust and would ordinarily be considered finished, I raise the filament to a very high temperature for a considerable time, say from three to ten minutes, by means of applying to it a voltage 105 very much in excess of its normal voltage. Toward the end of this operation and while the lamp is still at this high temperature, I

allow a small quantity of a gas or vapor such as phosphorus vapor to enter into the lamp. This I usually accomplish by the previous introduction of a small quantity of phosphorus into the tube which serves for exhausting the lamp, and I vaporize the phosphorus by heating it by means of a small torch. The phosphorus then seems to act upon the material in the way above described and to produce a smooth highly efficient surface.

The process may be repeated in some instances for obtaining a more thorough treatment, but usually this is not necessary.

I do not wish to confine myself to the specific material phosphorus as I find in practice that various other materials, such for instance as arsenic, and sulfur, and the like may be employed, but thus far I have obtained the best results by the use of phosphorus.

I find that filaments thus made do not have to be afterward aged as the texture and structure of the filaments seem to be much more permanent than when made by the usual processes.

I claim as my invention:

1. The process of manufacturing metallic filaments for incandescent electric lamps, which consists in heating the filaments to a temperature in excess of their normal operating temperature in a vessel exhausted of air, and simultaneously acting upon the same by a gas or vapor serving to reduce the surface of the filament to a compact smooth condition.

2. The process of manufacturing metallic filaments for incandescent lamps, which consists in heating the filaments to a temperature materially higher than the operating temperature thereof in an atmosphere of

phosphorus for a sufficient length of time to change its surface characteristics.

3. The process of manufacturing filaments for incandescent lamps, which consists in heating the filaments to a temperature materially higher than the operating temperature thereof in an atmosphere of phosphorus for a period materially longer than is customary in the process of exhausting.

4. The process of treating a metallic incandescent lamp filament which consists in heating the same while evacuating the lamp in the presence of an atmosphere of phosphorus to a temperature materially in excess of its temperature when in normal use for a sufficient length of time to change its surface characteristics.

5. The process of treating a metallic incandescent lamp filament, which consists in applying to it while it is located in a vacuum a voltage materially in excess of that applied to it in normal use and subjecting it while so heated to an atmosphere of phosphorus.

6. The process of treating a tungsten incandescent lamp filament which consists in heating the same while evacuating the lamp to a temperature materially in excess of its temperature when in normal use and for an extended period, and simultaneously acting upon the same by a gas or vapor serving to reduce the surface of the filament to a compact smooth condition.

In testimony whereof, I have hereunto subscribed my name this 23rd day of November, 1910.

ROBERT H. HENDERSON.

Witnesses:

GEORGE P. SCHOLL,  
CHARLES E. KELLY.